

Patented Jan. 11, 1927.

## UNITED STATES PATENT OFFICE.

JAMES L. STEVENS, OF HAYDEN, ARIZONA.

## CONCENTRATION OF ORES.

No Drawing.

Application filed July 1, 1926. Serial No. 119,993.

This invention relates to the concentration of ores, minerals, and the like, by flotation, and has for its object the provision of certain improvements in the flotation processes, 5 and more particularly the froth flotation processes.

The present invention is based upon a discovery that improved results may be obtained by the use in flotation of certain organic nitrogenous compounds containing sulphur, in which the (N) nitrogen is in the form of (CN) cyanogen, and the (S) sulphur is in combination therewith, forming the radical SCN in compounds commonly 10 known as sulphocyanides (or sulphocyanates). In certain cases these compounds may have a formula of R SCN in which R is an organic radical, such as an alkyl radical.

20 While the general formula of R SCN is given to show the constituents of the compounds covered by this specification, the scope of this invention in its broadest aspect is not limited to any particular method 25 of chemical combination nor to any particular structural formula or arrangement of atoms in the molecule, as I have found that various reaction products possessing valuable flotation properties and also possessing 30 various chemical and physical properties have resulted from various means of reaction as is hereinafter described.

Alkyl sulphocyanates (or sulphocyanides) 35 may be prepared by various wellknown methods; for example, I have prepared normal amyl sulphocyanate by distilling amyl sulphate with potassium sulphocyanate. The distillate from this mixture was 40 of an oily character, only slightly soluble in water and giving a deep red reaction with ferric sulphate. This compound, when employed as a flotation reagent for recovery of the metalliferous constituents 45 from the gangue minerals of an ore pulp, produced a voluminous, well mineralized froth, exhibiting a very marked selective action 50 on sulphide minerals. This compound apparently functions best when used in conjunction with a small amount of an acid (for example, sulphuric acid).

55 Amyl sulphocyanate possesses valuable frothing properties. The frothing properties of this compound, together with its marked selective action on sulphide minerals, enable the froth flotation process to be

successfully carried out without the employment of foreign frothing agents, such as pine oil or the like. For example, an ore pulp containing about 1.24% copper was subjected to agitation, and acid ( $H_2SO_4$ ) 60 added at the rate of 4 pounds per ton of solids. Amyl sulphocyanide was then added at the rate of about .8 lb. per ton of solids. Upon adding the amyl sulphocyanide a 65 voluminous, heavily mineralized froth was formed, which was removed from the gangue pulp by allowing same to overflow the flotation cell. The concentration in this operation was sufficient to reduce the tailings to 0.10% copper and produce a concentrate containing about 18.0% copper. This operation was conducted without the aid of a foreign frothing agent.

Various wellknown methods may be employed to produce normal alkyl sulphocyanides, which have the general formula R—S—C≡N. In these compounds the cyanogen radical is linked to the alkyl radical by sulphur. However, I have found that various compounds possessing valuable flotation 75 properties may be obtained by introducing the sulphocyanide radical (SCN) into various organic compounds by a simple method 80 of interaction of an acid. For example, I have found that by first treating an alcohol with an acid, such as, for example, sulphuric acid, or commercial aqueous hydrochloric acid, and adding to this mixture a salt of sulpho-cyanic acid, such as potassium sulphocyanate (K CNS) and subjecting the 85 mixture to various degrees of heat, say from atmospheric temperature up to the boiling 90 temperature of the compound, various chemical products may be formed, some of which 95 do not possess the properties of normal alkyl sulphocyanides and yet possess valuable flotation properties. For example, 98 parts by weight of concentrated sulphuric acid were slowly added to 74 parts by weight of 100 butyl alcohol. Considerable heat of reaction was produced by this mixture. The mixture was cooled and 97 parts by weight of potassium sulphocyanate in crystalline form added thereto. The mixture was agitated and diluted with 100 parts by weight 105 of water. The resultant product from this mixture was very soluble in water, and while this compound showed no evidence of the presence of normal butyl sulphocyanide, it possessed a marked selective action on sul-

phide minerals when used in the customary flotation processes. A flotation test conducted on an ore pulp, using the above diluted product at the rate of about .5 lb. per ton of solids, and pine oil at the rate of about .15 lb. per ton, gave the following metallurgical results:

| Heading      | Per cent copper |
|--------------|-----------------|
| 19 Tailings  | 0.11            |
| Concentrates | 11.30           |

In other tests in which I have employed acid for the purpose of combining or associating the radical of sulphocyanide (SCN) with alcohols, the following procedure was used: Mixtures of sulphuric acid and alcohols were brought to a boiling temperature and then cooled. Potassium sulphocyanate in crystalline form was then added. The mixtures were then heated gently and shaken until a homogeneous, pasty mass was formed. At this stage of the operation, in most cases, a small amount of an insoluble oily substance was formed. Both the oily material (alkyl sulphocyanide or similar substance) and the water soluble portion of the mixtures exhibited a very marked selective action on sulphide minerals. The mixtures were then subjected to additional heat and distilled. The distillate from these mixtures contained a large amount of the oily substance which resembled alkyl sulphocyanides in many respects, and exhibited a very marked selective action on metalliferous minerals, particularly sulphide minerals.

As an example of the above procedure, 100 parts of denatured ethyl alcohol (formula No. 5) were treated with 98 parts by weight of concentrated sulphuric acid. The mixture was heated to a boiling temperature and then cooled in an ice bath. 97 parts by weight of potassium sulphocyanate in crystalline form were then added. The mixture was heated gently, agitated until a homogeneous paste was formed; and then distilled. This method of combination has been applied to various other alcoholic compounds, for example, propyl, butyl, and amyl alcohols, the products of which were similar in each case to the above described compounds.

From the foregoing example, it is seen that an excess of alcohol, above the theoretical amount required for the reaction, was used. This excess of alcohol was used in order to prevent the presence of any large amount of free acid, as the reaction between the acid and alcohol is a reversible one, especially when subjected to heat. In general, therefore, it is advisable to use an excess of alcohol and reduce the mixture of alcohol and acid to a low temperature prior to adding the potassium sulphocyanate. An excess of free acid in the mixtures should be

avoided as far as possible as the free acid may cause complete decomposition of the potassium sulphocyanate



70

the products of which have little, if any, selective value as flotation agents.

I have also found that sulphocyanide may be advantageously introduced into (combined or associated with) various organic bodies such as frothing oils which may in some cases be lacking in selective properties. Such organic compounds, after the introduction of the sulphocyanide, possess a very marked selective action and may be caused to be very effective in separating the metalliferous minerals from the gangue minerals by flotation. As an example of this, I have introduced sulphocyanide into pine oil. Approximately 300 parts by weight of pine oil were treated with 98 parts by weight of sulphuric acid. Considerable heat was produced by this mixture and no additional heat was applied. The mixture, after being agitated a few minutes, was cooled, and 97 parts by weight of potassium sulphocyanate added. The mixture was thoroughly shaken and allowed to stand about one hour and then distilled. The complex compounds or mixtures contained in the distillate from this procedure possessed marked selective properties as well as the ordinary frothing properties of the pine oil.

75

I have also caused sulphur and cyanogen to be introduced into or combined with creosol or cresylic acid, which is also a frothing oil, and have found that products having the properties of sulphocyanides may be so produced and that these products give good results in flotation operations. For example, I have treated 300 parts by weight of cresylic acid with 98 parts by weight of sulphuric acid, and have then treated the product of this reaction, after a short agitation followed by cooling, with 97 parts by weight of potassium sulphocyanate. The mixture was shaken and allowed to stand and then distilled. The resulting distillate showed distinctive selective properties when used in flotation operations, in addition to the ordinary frothing properties of the cresylic acid.

80

From the foregoing examples, it is seen that my invention in its broadest sense contemplates the use in flotation of organic compounds containing a radical of sulphocyanide. More specifically, the invention contemplates on the one hand, the use in flotation of normal sulphocyanide compounds having the general formula  $R - S - C \equiv N$ , in which R may represent an alkyl or other organic radical, such as the radicals contained in pine oil; and on the other hand, the use of agents formed by the combination of the

85

90

95

100

105

110

115

120

125

sulphocyanide radical with an alkyl radical, or by the introduction of the sulphocyanide radical into frothing oils, such as pine oil, whether or not the resulting compounds are 5 normal sulphocyanides.

The following table shows the metallurgical results of flotation tests conducted on samples of ore pulp from the Ray Consolidated Copper Company, at Hayden, Arizona.

10 The various materials into which the sulphocyanide was introduced, (a) ethyl alcohol, (b) propyl alcohol, (c) butyl alcohol, (d) amyl alcohol, (e) fusel oil, (f) pine oil, and (g) cresylic acid, were treated with sulphuric acid, potassium sulphocyanide added, and the mixtures distilled as has previously 15 been described. The tests were conducted with the distillate in each case.

20 *Table of metallurgical results.*

| Test.     | Heads,<br>% Cu. | Rougher<br>tailings,<br>% Cu. | Rougher<br>concts.,<br>% Cu. |
|-----------|-----------------|-------------------------------|------------------------------|
| 25 a..... | .94             | .08                           | 5.6                          |
| b.....    | .98             | .18                           | 7.9                          |
| c.....    | .96             | .06                           | 5.7                          |
| d.....    | .96             | .07                           | 5.5                          |
| e.....    | .96             | .05                           | 5.5                          |
| f.....    | 1.00            | .14                           | 6.0                          |
| g.....    |                 | .11                           | 12.4                         |

30 Note: Pine oil was added in tests *a* and *b*. Tests *c*, *d*, *e*, *f*, and *g* were conducted without the aid of additional frothing agents. Tests *a*, *b*, *c*, *d*, *e*, and *g* were conducted in a pulp made slightly acid with sulphuric acid. Test *f* was conducted in an alkaline pulp.

35 I have specified potassium sulphocyanate as a source of obtaining the (SCN) sulphocyanide. The sulphocyanide may, however, be derived from any suitable source. I have for example, employed sodium sulphocyanate as a substitute for the potassium sulphocyanate.

40 45 I have described, in detail, several methods which may be employed in making the flotation agents herein described, however, any suitable method of combination or reaction may be used.

50 The chemical and physical properties of the compounds covered by this specification may vary over a wide range. For example, in some cases, the compounds are very oleaginous, while in other cases they are non-oleaginous. Also in some cases the compounds possess valuable frothing properties together with their marked selective action. In some cases these compounds do not possess frothing properties, and it is necessary to 55 supplement their selective action with a frothing agent. Furthermore, these compounds possess various degrees of solubility co in water, ranging from compounds that are readily and completely soluble in water to 65 compounds that are substantially insoluble in

water. Essentially, however, these compounds must contain sulfur and cyanogen substantially as described.

In applying the reagents herein described, they may be introduced into the ore pulp in 70 any suitable way; for instance, they may be introduced into the tube mill in which the ore is being ground or may be added to the ore pulp just before it enters the flotation cell. In general, however, I prefer to subject the reagents to agitation with the ore pulp prior to entering the flotation cell. 75

The amount of the reagents of the present invention, required for effecting the concentration of ores may vary somewhat. For 80 example, in treating ordinary clean sulphides the amount may be varied from  $\frac{1}{10}$  pound or less per ton of ore, to approximately one pound per ton of ore. In treating mixed 85 ores, such as ores containing sulphide and oxide metalliferous minerals, it may be advisable to use a larger quantity than is required for clean sulphide ores.

The reagents herein described may be employed as flotation agents in acid, neutral or alkaline ore pulps. In general, however, I prefer to employ these reagents in the presence of an acid electrolyte, such as, for example, sulphuric acid. Other neutral or acid electrolytes, such as calcium sulphate, acid 95 or neutral sodium or potassium sulphates in solution with water, may be added in any suitable manner. Thus the alkali metal salts derived from reactions in the formation of some of the compounds of the present invention may advantageously be employed in conjunction with the selective agents, thereby 100 reducing the additional quantities of acids or salts required, and also eliminating the necessity of segregating or purifying the 105 products of reaction. The acid may be added to the ore pulp before or after adding the selective agent.

In general, it is characteristic of the compounds of the present invention to cause 110 the mineral particles to be firmly attached to the bubbles forming the froth, and in this respect showing a more intimate relation between the action of these compounds on the surface of the mineral particles and the froth, than has been noticed with other compounds previously employed.

115 It will be understood by those skilled in the art that the present invention is applicable to the treatment by flotation of various kinds of mineral mixtures, both natural and artificial. In the appended claims I have accordingly employed the term "mineral pulp" in a broad sense to include mineral 120 products and all materials amenable to concentration or similar treatment by the flotation processes.

125 While I have mentioned the marked selective action of these compounds upon sulphide minerals, the results obtained by 130

their use in flotation have also indicated a strong selection for oxidized metalliferous minerals.

I claim:

- 5 1. The method of concentrating minerals which comprises adding to the mineral pulp a normal sulphocyanide of an organic compound and then subjecting the pulp to a froth flotation operation.
- 10 2. The method of concentrating ores or other materials which consists in treating a pulp containing such material with the reaction product produced by heating together an alkali sulphocyanide with an organic salt, and subjecting the pulp so treated to a froth flotation operation.
- 15 3. The method of concentrating minerals which comprises adding to the mineral pulp an alkyl sulphocyanide compound and then subjecting the pulp to a froth flotation operation.
- 20 4. The method of concentrating minerals which comprises adding to the mineral pulp a sulphocyanic ester of a higher alcohol and then subjecting the pulp to a froth flotation operation.
- 25 5. The method of concentrating minerals which comprises adding to the mineral pulp a flotation agent comprising butyl sulphocyanide and then subjecting the pulp to a froth flotation operation.
- 30 6. The method of concentrating ores or other material which consists in treating a pulp containing such materials with a compound containing an alkyl radical together with sulfur and cyanogen and then subjecting the pulp to a froth flotation operation.
- 35 7. The method of concentrating ores or other material which consists in adding to a pulp containing such material, an organic compound containing sulfur and cyanogen, and subjecting the pulp to froth flotation in the presence of such compound.
- 40 8. The method of concentrating minerals which comprises adding to the mineral pulp

a flotation agent produced by treating an alcohol with acid and with a sulphocyanate salt, and then subjecting the pulp to a froth flotation operation.

9. The method of concentrating minerals 50 which comprises adding to the mineral pulp a flotation agent produced by treating an alcohol with sulphuric acid and with a sulphocyanate salt, and then subjecting the pulp to a froth flotation operation. 55

10. The method of concentrating minerals which comprises adding to the mineral pulp a flotation agent produced by treating a higher alcohol with acid and with a sulphocyanate salt, and then subjecting the pulp to 60 a froth flotation operation.

11. The method of concentrating minerals which comprises adding to the mineral pulp a flotation agent produced by treating butyl alcohol with acid and with a sulphocyanate 65 salt, and then subjecting the pulp to a froth flotation operation.

12. The method of concentrating minerals which comprises adding to the mineral pulp a normal sulphocyanide of an organic compound and also adding thereto an electrolyte, and then subjecting the pulp to a froth flotation operation. 70

13. The method of concentrating minerals which comprises adding to the mineral pulp 75 an organic sulphocyanide compound and also adding thereto an acid electrolyte, and then subjecting the pulp to a froth flotation operation.

14. The method of concentrating minerals 80 by flotation which comprises adding to the mineral pulp an alkyl sulphocyanide compound, and also adding thereto an electrolyte, and then subjecting the pulp to a froth flotation operation. 85

15. The method as set forth in claim 14, said electrolyte being an acid electrolyte.

In testimony whereof I have hereunto subscribed my name this 25th day of June 1926.

JAMES L. STEVENS.